

April 26, 1938.

W. H. HAMPTON ET AL.

2,115,306

ASPHALTIC MATERIAL AND PROCESS FOR PRODUCING THE SAME

Filed Aug. 11, 1934

2 Sheets-Sheet 1



Fig. 1



Fig. 2



Fig. 3

Inventors

WILLIAM H. HAMPTON

ORVILLE E. CUSHMAN

JOSEPH E. FRATIS

by

*W. H. Hampton*  
Attorney

April 26, 1938.

W. H. HAMPTON ET AL.

2,115,306

ASPHALTIC MATERIAL AND PROCESS FOR PRODUCING THE SAME

Filed Aug. 11, 1934

2 Sheets-Sheet 2



Fig. 4



Fig. 5



Fig. 6

*Inventors*

WILLIAM H. HAMPTON

ORVILLE E. CUSHMAN

JOSEPH E. FRATIS

by *W. H. Hampton*  
Attorney

## UNITED STATES PATENT OFFICE

2,115,306

ASPHALTIC MATERIAL AND PROCESS FOR  
PRODUCING THE SAME

William H. Hampton, Orville E. Cushman, and  
Joseph E. Fratis, Berkeley, Calif., assignors to  
Standard Oil Company of California, San  
Francisco, Calif., a corporation of Delaware

Application August 11, 1934, Serial No. 739,448

10 Claims.

(Cl. 260—2)

This invention relates to a new composition of matter and more particularly to a synthetic plastic material, which for convenience in identification by comparison and contrast with petroleum and natural asphalts may be called a synthetic asphalt, and to a method for preparing the same.

It has long been known that the gaseous olefins and diolefins containing from two to about five carbon atoms can be caused, by appropriate means, to polymerize into various liquid and solid materials. It has more recently been learned that by proper choice of the gaseous raw material, of the physical conditions of pressure, temperature and time and finally of the contact material or catalyst employed that the nature of the polymerization product can be predetermined within certain limits. This knowledge has in the very recent past been applied in a considerable number of processes to a utilization of the gaseous unsaturates consisting chiefly of olefins produced during the cracking of petroleum oils in the production of motor fuels.

By the appropriate polymerization of these low molecular weight olefins low boiling compounds in the range of motor fuels, intermediate boiling fractions such as transformer oils, cosmetic oils, etc., and high boiling stocks in the boiling range of lubricating oils and cylinder oils are now being produced on a considerable scale. As was to have been expected these synthetic products differ markedly in many respects from the similar boiling distillates from petroleum.

We have now discovered that by still further treating certain of these heavier olefin polymers by subjecting them to what is broadly a process of oxidation an entirely new group of materials may be produced, which we have chosen to call synthetic asphalts. These materials may be produced with varying degrees of hardness and with melting or softening points variable throughout a considerable range depending upon the nature of the olefine polymer material oxidized and the extent to which oxidation is carried. They are apparently supercooled liquids as distinguished from true solids and hence may be subjected to and identified by the same set of physical tests as are customarily applied to natural and petroleum asphalts.

It is the broad object of this invention to produce a synthetic plastic of desirable characteristics from gaseous olefins.

It is a further object of this invention to produce a synthetic asphalt-like material from gase-

ous olefins through the successive reactions of polymerization and oxidation.

Another object of our invention is to produce a synthetic asphalt-like material whose physical characteristics may be predetermined within 5 rather wide limits.

Still another object of our invention is to produce an asphalt-like material whose physical properties change but little with changes in temperature.

A further object of our invention is to produce a synthetic asphalt-like material which is extremely resistant to subsequent attack either by chemical agencies or by the atmospheric agencies which contribute to weathering.

Still other objects will become apparent from the description and discussion of our process and product which follow.

Our process consists broadly in first preparing heavy olefin polymers of boiling points in the range of lubricating oils or above by any suitable means and of then subjecting them to oxidation by one of the more powerful oxidizing materials such as oxygen, sulfur or chlorine. In its simplest embodiment we prepare a suitable olefine polymer liquid and subject it to the action of air in any appropriate container maintaining the temperature within the desired range by the application of heat from any suitable external source. Oxidation is continued until a sample of the product drawn from the apparatus shows the desired characteristics. Oxidation need not necessarily be confined to a single oxidizing agent. Air and sulfur used together may often yield a product which is more desirable than that produced by either alone.

The temperature of oxidation with air will vary between about 300° F. and 500° F. and may advantageously be started somewhere near the lower limit and progressively raised as the oxidation proceeds. Operation with sulfur as the oxidizing agent is very similar while when chlorine is employed the conditions may have to be varied somewhat in order to secure the proper absorption of chlorine and its re-emission as hydrogen chloride.

Usual precautions should be observed to prevent excessive local or skin temperatures at any time during the reaction since the inclusion of even small amounts of cracked products would in most cases confer upon the synthetic asphalt properties which would be highly undesirable and in no sense characteristic of the synthetic product itself.

The following specific example will serve to 55

illustrate our method and to show how it may be carried out. We first polymerize the olefins contained in a cracking still gas by subjecting them to the action of a polymerizing catalyst such as aluminum chloride or strong sulfuric acid. Usually, though not necessarily, the olefins will be employed in liquefied form and the catalyst in solution. Having thus prepared an olefine polymer liquid with a viscosity of about 1000 seconds Saybolt universal at 210° F. and freed it from any residual catalyst we next charge it to a still equipped for the introduction of air and similar in general to the stills employed in the preparation of air-blown petroleum asphalts.

Having raised the temperature of the liquid polymers to about 300° F. a current of air is admitted and the temperature is increased at a rate of about 1° F. per hour so that at the end of 150-170 hours the temperature of the still contents will have reached about 450° F. If oxidation is discontinued at this point a material giving the tests recorded in column 3 of Table 1, which follows, will have been produced. The materials of columns 1 and 2 of this table resulted from somewhat less oxidation while column 4 contains results on a sulfur oxidized material.

beyond the limits that have ever been realized in materials prepared directly from petroleum ingredients as to clearly set it apart as a new composition of matter.

With regard to Figure 2 it should be noted that petroleum asphalts of melting point greater than 275° F. having an appreciable ductility are entirely unknown while our materials of 50° F. higher melting point still have very appreciable and highly useful ductilities. In connection with this same chart it should be pointed out that, as is well known in the industry, ductilities greater than 6 to 8 have very little meaning so that comparisons of higher figures are of no value.

Referring now to Figure 6 one of the reasons for our choice of the two specific air-blown petroleum asphalts recorded in Table 1 as #1 and #2 becomes apparent since #2 has a penetration at 115° F. and #1 at 77° F. substantially identical with the penetrations at these two temperatures of our #3 sample of air oxidized polymers.

Still another reason for the choice of air-blown asphalt #1 is apparent from Figure 3. This particular product is a commercial preparation designed especially for sealing storage batteries and is made by air-blowing a petroleum distillate instead of a residuum and since it is thus not strict-

Table 1

|                                          | 175 pen.<br>air-blown<br>polymers | 100 pen.<br>air-blown<br>polymers | 70 pen.<br>air-blown<br>polymers | 70 pen.<br>sulphur<br>oxidized<br>polymers | Air-blown asphalt |       |       |
|------------------------------------------|-----------------------------------|-----------------------------------|----------------------------------|--------------------------------------------|-------------------|-------|-------|
|                                          |                                   |                                   |                                  |                                            | 1                 | 2     | 3     |
| 35 Specific gravity                      | 0.9872                            | .951                              | .960                             |                                            | 1.005             | 1.037 | 1.050 |
| Pen. @ 77° F.                            |                                   |                                   |                                  |                                            |                   |       |       |
| 100 grams 5'                             | 175                               | 104                               | 74                               | 69                                         | 75                | 30    | 14    |
| Pen. @ 32° F.                            |                                   |                                   |                                  |                                            |                   |       |       |
| 200 grams 60'                            | 181                               | 125                               | 99                               | 86                                         | 16                | 18    | 12    |
| Pen. @ 115° F.                           |                                   |                                   |                                  |                                            |                   |       |       |
| 50 grams 5'                              | 210                               | 124                               | 74                               | 80                                         | 230               | 72    | 22    |
| 40 M. P. ball and ring, °F.              |                                   |                                   |                                  |                                            |                   |       |       |
| Flash                                    | 175                               | 255                               | 320                              | 320                                        | 178               | 176   | 238   |
| Sol. CCl <sub>4</sub>                    | 520                               | 480                               |                                  |                                            | 510               | 435   | 420   |
| Sol. 86° gas                             | 99.9                              | 99.9                              | 92.6                             |                                            | 98.6              | 99.9  | 99.9  |
| Percent fixed carbon                     | 99.9                              | 91.7                              | 71.7                             |                                            | 67.8              | 61.2  | 58.0  |
| Loss by evaporation, 100 hours @ 325° F. | 3.8                               | 5.4                               | 5.0                              |                                            | 12.9              | 13.1  | 12.6  |
| Penetration after heating                | 0.0                               | 0.0                               | 0.0                              |                                            | 0.10              | 0.63  | 0.30  |
| Ductility @ 77°                          | 169                               | 101                               | 72                               |                                            | 72                | 28    | 14    |
| 45 Ductility @ 32°                       | 7.5                               | 3.5                               | 2.5                              | 3.0                                        | 2.75              | 5.0   | 1.0   |

Since our oxidized polymers resemble somewhat air-blown petroleum asphalts we have included in this same table for comparison the results of tests on three air-blown petroleum products. However, except for illustrating some specific point or points of similarity or difference, such tables of figures are of little value. In order therefore that the novel characteristics of our new synthetic material may be more easily appreciated and visualized the attached drawings are presented. In Figures 1 to 5 various functions, penetration, ductility, specific gravity, solubility in 86° naphtha and fixed carbon are plotted against the melting point as determined by the customary ring and ball method. In Figure 6 penetrations at the three standard temperatures, 32, 77 and 115° F. are plotted against the temperature in order to illustrate the low susceptibility of our product to temperature change and to contrast this important property with that of air-blown petroleum asphalts.

In Figures 1-5 inclusive the shaded areas have been made to include the extremes, so far as we have been able to compile them, for air-blown petroleum products from crude oils of a sufficiently wide range of characteristics as to include substantially all air-blown asphalts.

In each instance the physical properties of our synthetic material fall so far outside of and be-

ly an air-blown asphalt it might be expected to show as wide a departure in physical properties from a true air-blown asphalt as it would be possible to prepare from the ingredients of a natural petroleum. It, however, falls without the shaded area of air-blown asphalts on only this one chart, specific gravity vs. melting point, falling well within this area on all the other charts.

While we have been unable to find any such it appears entirely possible that still other petroleum derivatives may have been or might be specially prepared which would have properties that would fall without the shaded area of some one or other of the charts. It would however seem highly improbable that any such material has been or could ever be obtained from the components of a natural petroleum which would fall substantially without the shaded areas of two or more of the charts and certainly not without all of them as do our synthetic materials.

It will be noted that in Figures 1-5 we have indicated the respective properties of our synthetic asphalts by lines rather than by areas as there seems every reason to expect that they would have been had the values for a very large number of samples prepared under the widest possible range of operable conditions been available in preparing the charts as was the case with the air-blown asphalts. It is to be understood therefore

that we consider the material of our invention to be entitled to a reasonable range of equivalents of which the lines drawn may be taken as the average.

- 5 Other than the physical properties of our synthetic asphalts which set them apart from the closest hitherto known preparations are certain of their chemical characteristics chief among which is probably their striking unreactivity.
- 10 The very fact that it takes 150 to 170 hours of oxidation to prepare a product of 70 penetration whereas the usual 70 penetration air-blown asphalts are prepared under similar conditions in 20-30 hours or less is indicative of this feature.
- 15 It is however more specifically indicated and may be roughly evaluated from tests carried out in the "weatherometer", an apparatus which is familiar in the protective coating industry. Test samples coated with asphaltic paints prepared from the best air-blown asphalts obtainable and from our synthetic asphalts were run at the same time. The petroleum asphalt paints showed very considerable decomposition at the end of three complete "cycles" while paints prepared from our synthetic product showed no deterioration whatever after fifty complete "cycles" which is the equivalent of a year or more of exposure to ordinary atmospheric weathering.

This same unreactivity coupled with a low dielectric constant, high dielectric strength and a low susceptibility to temperature changes all combine to give a product which is highly desirable for many uses as an electrical insulating material.

- 35 We have further found that the several characteristics of our synthetic asphalts are so pronounced that when they are blended in even minor proportions with petroleum asphalts, products of very superior properties for certain specific uses are obtained. For instance a blend of 25% of our product with an ordinary air-blown petroleum asphalt will produce a base for an asphaltic paint which is far superior in its ability to withstand weathering to any asphaltic paint prepared wholly from petroleum asphalt or petroleum asphalt in admixture with natural asphalts or asphaltites.

Still other desirable uses to which our product may be put will be readily apparent to those skilled in the arts from the novel properties which have been given.

50 The term "olefin" is used herein in its strict chemical sense to mean solely an aliphatic hydrocarbon having one carbon to carbon double bond per molecule.

55 Having now described our new product and the methods by which it may be prepared what we claim is:

1. The method of producing a synthetic asphalt-like hydrocarbon plastic which comprises polymerizing normally gaseous olefins by means of anhydrous aluminum chloride followed by subjecting the heavy liquid olefin polymers so produced to oxidation by blowing with air at a temperature above 300° F. until a plastic solid product is produced.

2. The method of producing a synthetic asphalt-like hydrocarbon plastic which comprises polymerizing normally gaseous olefins by means of anhydrous aluminum chloride, separating a fraction of the polymerization product having a viscosity above about 500 seconds Saybolt universal at 210° F., subjecting such fraction to oxidation at a temperature above about 300° F., but below a temperature at which appreciable ther-

mal cracking would occur and continuing such oxidation until a plastic having a melting point above ordinary atmospheric temperature is obtained.

3. The method of producing a synthetic asphalt-like hydrocarbon plastic which comprises polymerizing normally gaseous olefins by means of a polymerization catalyst selected from the group consisting of strong sulfuric acid and aluminum chloride, followed by subjecting the heavy liquid olefin polymers so produced to oxidation by blowing with air at a temperature above 300° F. until a plastic solid product is produced.

4. The method of producing a synthetic asphalt-like hydrocarbon plastic which comprises polymerizing normally gaseous olefins by means of strong sulfuric acid followed by subjecting the heavy liquid olefin polymers so produced to oxidation by blowing with air at a temperature above 300° F. until a plastic solid product is produced.

5. The method of producing a synthetic asphalt-like hydrocarbon plastic which comprises polymerizing normally gaseous olefins by means of a polymerization catalyst selected from the group consisting of strong sulfuric acid and aluminum chloride, separating a fraction of the polymerization product having a viscosity above about 500 seconds Saybolt universal at 210° F., subjecting such fraction to oxidation at a temperature above about 300° F., but below a temperature at which appreciable thermal cracking would occur and continuing such oxidation until a plastic having a melting point above ordinary atmospheric temperatures is obtained.

6. The method of producing a synthetic asphalt-like hydrocarbon plastic which comprises polymerizing normally gaseous olefins by means of strong sulfuric acid, separating a fraction of the polymerization product having a viscosity above about 500 seconds Saybolt universal at 210° F., subjecting such fraction to oxidation at a temperature above about 300° F., but below a temperature at which appreciable thermal cracking would occur and continuing such oxidation until a plastic having a melting point above ordinary atmospheric temperatures is obtained.

7. The method of producing a synthetic asphalt-like hydrocarbon plastic which comprises polymerizing normally gaseous olefins by subjecting them to the action of a polymerization catalyst such as aluminum chloride or strong sulfuric acid, separating a fraction of the polymerization product having a viscosity above about 500 seconds Saybolt universal at 210° F., subjecting such fraction to oxidation at a temperature above about 300° F., but below a temperature at which appreciable thermal cracking would occur and continuing such oxidation until a plastic having a melting point above ordinary atmospheric temperatures is obtained.

8. A synthetic asphalt-like hydrocarbon plastic as prepared by the process of claim 2 which has a ductility greater than 1.0 at a melting point of 320° F. and having ductilities progressively greater than 1.0 at melting points below 320° F. being 6.5 or above at a melting point of 175° F., which has a penetration at 77° F. of 50 or above for a melting point of 320° F. and having penetrations progressively greater than 50 for melting points below 320° F. being 140 or above at a melting point of 175° F., which has a fixed carbon content of less than 9 for all melting points up to 75

to and including 320° F., and which has a specific gravity less than 0.98 for all melting points up to and including 320° F., and which has a solubility in 86° naphtha greater than 70% for a melting point of 320° F. and progressively greater at lower melting points approaching 100% at a melting point of 175° F.

9. A synthetic asphalt-like hydrocarbon plastic as prepared by the process of claim 5 which has a ductility greater than 1.0 at a melting point of 320° F. and having ductilities progressively greater than 1.0 at melting points below 320° F. being 6.5 or above at a melting point of 175° F., which has a penetration at 77° F. of 50 or above for a melting point of 320° F. and having penetrations progressively greater than 50 for melting points below 320° F. being 140 or above at a melting point of 175° F., which has a fixed carbon content of less than 9 for all melting points up to and including 320° F., and which has a specific gravity less than 0.98 for all melting points up to and including 320° F., and which has a solubility in 86° naphtha greater than 70% for a melting point of 320° F. and progressively greater

at lower melting points approaching 100% at a melting point of 175° F.

10. A synthetic asphalt-like hydrocarbon plastic as prepared by the process of claim 7 which has a ductility greater than 1.0 at a melting point of 320° F. and having ductilities progressively greater than 1.0 at melting points below 320° F. being 6.5 or above at a melting point of 175° F., which has a penetration at 77° F. of 50 or above for a melting point of 320° F. and having penetrations progressively greater than 50 for melting points below 320° F. being 140 or above at a melting point of 175° F., which has a fixed carbon content of less than 9 for all melting points up to and including 320° F., and which has a specific gravity less than 0.98 for all melting points up to and including 320° F., and which has a solubility in 86° naphtha greater than 70% for a melting point of 320° F. and progressively greater at lower melting points approaching 100% at a melting point of 175° F.

WILLIAM H. HAMPTON.  
ORVILLE E. CUSHMAN.  
JOSEPH E. FRATIS.